

## UNITED STATES PATENT OFFICE

2,556,686

## METHOD OF DRYING HARDWOOD

Armin Elmendorf, Winnetka, Ill.

No Drawing; Application October 16, 1946;  
Serial No. 703,460

2 Claims. (Cl. 34—12)

1

Thin wood boards or sheets, properly dried from a green state while constrained against shrinkage in width during drying, possess certain desirable properties. Although there is a slight contraction in width upon release of the wood at the end of the drying operation, the wood will not expand nearly so much as does like wood, that was not constrained during drying, when both afterwards absorb moisture. Consequently, in situations where the swelling of wood upon taking up moisture may cause trouble, it is of advantage to use wood that has been dried under constraint. Thus, for example, hardwood floor coverings made of ordinary, normally dried wood from .10 to .20 inch thick, bonded to an underlying sub-floor, frequently buckle or bulge upon taking up moisture; whereas such floors, if made of wood successfully dried under constraint in manufacture, will stay down and remain flat under the same conditions.

Manufacturing experience has shown that when hardwoods, such as oak and walnut, are dried from a green state under heat and pressure while constrained against shrinkage across the width of the board or sheet (in a ventilated hot press as, for example, shown in my Patent 2,268,477) they are frequently so badly damaged by the drying as to be unfit for use in the manufacture of floor coverings. The damage caused in drying is often not evident in the surface and is revealed only when the wood is sanded and considerable expense has been incurred in fabrication.

The defects in wood caused by drying it under constraint, while being subjected to heat, are generally visible on the surface as dark areas where the wood has been reduced in thickness due to partial hydrolysis of the cellulosic components of the wood. In such areas some of the cellulose has been converted into soluble sugars, so that the presence of the highly objectionable hydrolysis is also revealed by an odor as of overheated caramel. The density of the dark hydrolyzed areas exceeds that of the normal wood and, instead of being harder, the wood is easily gouged. As partial hydrolysis over some areas is very frequent, the resultant loss due to damage in drying is very great.

The presence of hydrolysis is frequently not visible from the surface as it may take place only in the interior of the board. In that case the wood is excessively honeycombed and sanding the surface preparatory to finishing may reveal the damage. When this happens, not only is the wood lost because it cannot be used

2

for flooring, but considerable labor in manufacture has also been lost.

I have discovered that the damage herein described is always associated with the expulsion of free moisture in the wood, and that it can be controlled. Due to differences in structure of the wood itself, in different areas of the same board, it appears that in some areas the moisture becomes trapped soon after the conversion into steam begins, and it is the pressure of pockets of high pressure steam that causes the hydrolysis. In order to dry the wood successfully while held under constraint, it is therefore necessary that the drying be done in such a manner that the steam pockets are not formed.

Many trials were made in a commercial operation in endeavors to find those conditions, if there were any, which would prevent the formation of steam pockets in the wood. Attempts 20 were made partially to dry thin oak boards freely, as in air drying or kiln drying, down to the fiber saturation point as revealed by incipient shrinkage, to remove free moisture, and then completing the drying under constraint; but, while hydrolysis under those conditions was not so prevalent, it was still sufficiently frequent to cause considerable loss of boards. Additional trials, drying freely still further, proved that the wood must be dried without constraint until appreciable shrinkage has taken place before hydrolysis is reduced to a satisfactory minimum. It was finally established that the critical point is reached when free drying is continued until a shrinkage in width from 1% to 3% has taken place, further drying then being under constraint so that no additional reduction in width occurs, with the exception of that due to elastic contraction upon removal of the constraint.

It appears that when a board is dried without constraint to the state at which shrinkage in width to the extent of from 1% to 3% occurs, the moisture content of the center of the same is at or near the fiber saturation point while the moisture of the surface fibers is below the fiber saturation point; which condition may be used as a basis to determine when drying under constraint should begin, although not as easy to measure as the amount of shrinkage in width.

Drying under constraint may continue until the moisture in the wood is reduced to from 1% to 5%. It is preferable that the boards be dried under constraint to practically bone-dry conditions and then have their moisture raised to the desired 6% to 8%; the addition of moisture being effected through exposure to high humid-

ties in a humidified enclosure, or through momentary submersion in water, followed by cooling and evaporation of the excess moisture.

The fact that some shrinkage has already taken place at the end of the first drying stage makes it possible quickly and accurately to determine when that stage should end. In other words, it is a simple matter to set a guage for any given lot of raw material, which is then dried in a conventional mechanical drier, or air dried, until it has shrunk to fit the guage and so is ready to be dried under constraint.

The resultant board, dried in two stages as described, possesses maximum width consistent with complete freedom from hydrolysis, it is flat, and, when slit and backed with a flexible backing, it is flexible and readily adjusts itself to unevenness in the sub-floor upon which it is laid. When, after bonding to the sub-floor, its moisture is increased, it expands much less than do similar boards dried by conventional procedures, and floor failures due to buckling are practically completely eliminated.

I claim:

1. The method of drying thin boards of hard wood in which objectionable hydrolysis frequently takes place when the same is dried from a green state to the state of stable moisture content, while held under constraint to prevent shrinkage and subjected to heat; which consists in drying such boards, without constraint, until the free moisture is removed from the interior thereof and the outside thereof is somewhat below the fiber saturation point, and then drying them under constraint to prevent shrinkage while being subjected to heat and pressure.

2. The method of drying thin boards of hard wood in which objectionable hydrolysis frequently occurs when the same is dried, from a green state to the state of stable moisture content while held under constraint to prevent shrinkage and heated; which consists in drying such boards without constraint until the free moisture has been removed from the interior thereof and they shrink from 1% to 3% in width, and then drying the same under constraint to prevent shrinkage while being subjected to heat and pressure.

ARMIN ELMENDORF.

#### REFERENCES CITED

The following references are of record in the file of this patent:

#### UNITED STATES PATENTS

| Number    | Name                | Date          |
|-----------|---------------------|---------------|
| 1,573,297 | Briner et al. ----- | Feb. 16, 1926 |
| 1,578,020 | Elmendorf -----     | Mar. 23, 1926 |
| 1,677,963 | Ford -----          | July 24, 1928 |
| 1,903,102 | Farley -----        | Mar. 28, 1933 |
| 1,909,213 | Munroe -----        | May 16, 1933  |
| 2,132,095 | Broughton -----     | Oct. 4, 1938  |
| 2,284,838 | Ohlom -----         | June 2, 1942  |

#### OTHER REFERENCES

30 The Kiln Drying of Lumber, by Koehler and Thelen, published 1926 by McGraw-Hill Book Co., New York, pages 42 and 46.

Drying and Processing of Materials by Carrier Engineering Corp., published 1929, page 181.